

## UNITED STATES PATENT OFFICE

2,607,665

## FUEL OIL COMPOSITION

Gordon W. Duncan, Westfield, N. J., assignor to Standard Oil Development Company, a corporation of Delaware

No Drawing. Application April 7, 1950,  
Serial No. 154,735

2 Claims. (Cl. 44—72)

## 1

The present invention relates to an improvement in fuel oils and more specifically to a method of decreasing the emulsification tendency of medium diesel fuel oils.

In selecting fuels for marine diesel engines, heavier and less refined products are generally desired because of their lower cost. Unfortunately, such fuels are especially susceptible to emulsification with water, and excessive emulsifiability results in placing an undue load on purifying devices such as centrifuges and filters and can result in accelerated diesel fuel pump and injector wear and corrosion. A compromise must be made to arrive at the least costly product which has adequate resistance to emulsion. In accordance with this invention, it is now possible to treat economically many high emulsifiability diesel fuels to render them entirely satisfactory in this respect. The fuels particularly suited to the practice of the invention are distillate products such as are generally termed "medium" diesel fuels, which through lack of refining tend to be unduly susceptible to emulsification on contact with water. The following inspection data better illustrate the type of fuel suitable for use:

|                               |      |
|-------------------------------|------|
| Gravity, A. P. I              | 29.5 |
| Viscosity at 100° F., S. U. S | 51.9 |
| Flash pt., °F                 | 192  |
| Aniline pt., °F               | 158  |
| Cetane No                     | 49   |
| Pour pt., °F                  | +10  |
| Sulfur, per cent              | 1.31 |
| Conradson carbon, per cent    | 1.38 |
| Ash, per cent                 | 0.01 |
| Neutralization No             | 0.19 |
| B. S. & W                     | 0.14 |

## Distillation characteristics at atmospheric pressure up to 700° F.

|         |     |
|---------|-----|
| I. B. P | 393 |
| 2%      | 428 |
| 5%      | 447 |
| 10%     | 465 |
| 20%     | 498 |
| 30%     | 527 |
| 40%     | 560 |
| 50%     | 595 |
| 60%     | 634 |
| 70%     | 674 |
| 78%     | 697 |

"Medium" diesel fuels are generally considered to be those with viscosities in the range of about 33 to 75 Saybolt Universal seconds at 100° F.

It has now been found that a low-pour, substantially residuum-free, highly emulsifiable fuel, unsatisfactory for marine use, may be rendered suitable for such use by the incorporation therein of small amounts of long chain (C<sub>10</sub>—C<sub>18</sub>) primary amines, i. e. decyl amine, undecyl amine, dodecyl amine, tridecyl amine, tetradecyl amine, pentadecyl amine, and hexadecyl amine.

Aromatic amines, aromatic hydroxy amines, hexyl amine, and benzidine have been previously proposed to stabilize the pour point of heavy, residual, wax-containing fuel oils. See U. S. 2,216,230 issued October 1, 1940, to G. H. B. Davis. However, these amines will not act to overcome the emulsifying tendencies of lighter fuel oils.

The amount of amines added in accordance with the present invention is not large, being not greater than 0.5% by weight. In some cases the addition of so little as 0.01% has a noticeable effect on the emulsifying tendency of an oil. Generally, a concentration of amine between 0.02 and 0.1% is employed, the range from 0.03 to 0.05% being preferred since in most cases this quantity will reduce the emulsifying tendency to a low level.

As an example of the use of the present invention, the following should be considered:

| Example |                 |                                         |                               |
|---------|-----------------|-----------------------------------------|-------------------------------|
|         | Fuel Used       | Conc. of Additive Weight Percent        | Relative Emulsifying Tendency |
| 35      | Medium Fuel Oil |                                         |                               |
|         | Do              | 0.005 Coco amine <sup>1</sup>           | 11.5                          |
|         | Do              | 0.01 Coco amine <sup>1</sup>            | 9.95                          |
|         | Do              | 0.01 Coco amine <sup>1</sup>            | 11.5                          |
|         | Do              | 0.01 Coco amine <sup>1</sup>            | 7.25                          |
|         | Do              | 0.02 Coco amine <sup>1</sup>            | 9.75                          |
|         | Do              | 0.05 Coco amine <sup>1</sup>            | 8.0                           |
|         | Do              | 0.1 Coco amine <sup>1</sup>             | 1.0                           |
|         | Do              | 0.1 Coco amine <sup>1</sup>             | 0.5                           |
|         | Do              | 0.1 Nonyl Amine                         | 1.0                           |
|         | Do              | 0.1 2H <sup>2</sup> Ammine <sup>2</sup> | 4.0                           |
|         | Do              | 0.1 Octadecenyl nitrile <sup>3</sup>    | 9.0                           |
|         | Do              | 0.1 AM-1180 <sup>4</sup>                | 8.5                           |
|         | Do              |                                         | 5.0                           |

<sup>1</sup> A mixture of C<sub>10</sub>—C<sub>16</sub> (principally C<sub>12</sub>—C<sub>14</sub>) primary saturated amines.

<sup>2</sup> A mixture of C<sub>16</sub>—C<sub>18</sub> secondary saturated amines.

<sup>3</sup> C<sub>18</sub> unsaturated cyanide.

<sup>4</sup> C<sub>18</sub> saturated primary amine.

From the above data it is evident that the aliphatic amines having 10—16 carbon atoms are eminently suitable for reducing the emulsion tendency of fuel oils, and are considerably superior to nonyl amine having nine carbon atoms, to C<sub>18</sub> saturated primary amine, and also to secondary amines having from 16 to 18 carbon atoms.

This invention also has application for use with fuel oils for domestic and industrial applications and in general for any lightly refined distillate fuel oil needing improved emulsification resistance.

The nature and objects of the present invention having been thus fully set forth, what is claimed as new and useful and desired to be secured by Letters Patent is:

1. An improved distillate marine diesel fuel substantially free of residual petroleum fractions and containing 0.05 to 0.10 per cent of a mixture of primary straight chain saturated aliphatic alkyl-amines having from 10 to 16 carbon atoms

and having a minimum tendency to cause emulsification of said fuel in water and of water in said fuel.

5 2. A composition as in claim 1 wherein the amines have from 12 to 14 carbon atoms.

GORDON W. DUNCAN.

#### REFERENCES CITED

The following references are of record in the file of this patent:

#### UNITED STATES PATENTS

| Number    | Name      | Date          |
|-----------|-----------|---------------|
| 2,246,842 | De Groote | June 24, 1941 |